

March 22, 1938.

A. M. TENNEY

2,112,123

FABRIC

Filed June 1, 1936



*Ashton M. Tenney*  
INVENTOR

BY *Newton M. Purvis*

ATTORNEY.

## UNITED STATES PATENT OFFICE

2,112,123

## FABRIC

Ashton M. Tenney, New Rochelle, N. Y., assignor,  
by mesne assignments, to Eastman Kodak Company,  
Jersey City, N. J., a corporation of New Jersey

Application June 1, 1936, Serial No. 82,860

8 Claims. (Cl. 139—426)

This invention relates to fabrics in which are used yarns of cellulose acetate and of mohair or other animal fibre, particularly of natural hair or wool.

5 It has long been known that animal fibres and particularly natural hair and wool have a spring or elasticity that is lacking in vegetable fibres such as cotton and filaments made from cotton derivatives, such as viscose or cellulose acetate.

10 This tends to render fabrics wrinkle resistant.

Natural fibres both of animal and vegetable origin, such as wool, mohair and cotton, as well as such artificial filaments as viscose, have also high water absorption and swell and shrink under 15 moisture and drying, the shrinkage of the rough fibres, such as wool or mohair, being particularly pronounced, because the fibres mat together to such an extent that the natural resilience of the fibre cannot again separate them.

20 Cellulose acetate, however, being highly water resistant, does not swell or shrink appreciably because of wetting and drying. Moreover it does not irritate the body of the wearer as do some woolen clothes.

25 This invention relates to a fabric in which the advantages of both types of yarn are obtained and the disadvantages minimized and comprises the use as warp of yarn solely or predominantly of cellulose acetate and as woof or filling of a 30 yarn containing both cellulose acetate and mohair or other animal fibre. The animal fibre gives body and resilience to the fabric, and the cellulose acetate counteracts the shrinking of the wool. The fabric is non-irritant and of pleasing 35 appearance.

35 Reference will be made to the drawing, the single figure of which shows in a conventional or diagrammatic manner a fabric involving my invention.

40 Certain threads, which may be warp threads, are indicated at 1 and the others, which may be the filling or woof threads, at 2. While a perfectly plain weave is shown, it is to be understood that any type or design may be used. These 45 warp threads are preferably of cellulose acetate only and may be continuous or spun threads.

One type of yarn which may be used for the warp is made in the following manner. The filaments are extruded and twisted in the usual manner to form a coherent thread or yarn. This is 50 preferably crimped and then abraded to such an extent that some of the outer filaments are broken, usually from 30 to 35 per cent of the filaments, although more or less may be. This 55 causes the threads to have a fuzzy or woolly sur-

face, especially if they have been crimped. A fabric containing such yarn and also yarn containing wool, angora, merino, cashmere, camel's hair, mohair or the like, has great covering power and body.

5 It is to be understood that other forms of cellulose acetate yarn may be used, and that these may be spun or be continuous or be twisted from two or more strands, but in any event this thread will be predominantly of cellulose acetate.

The filling threads 2, on the other hand, are 10 strands of cellulose acetate and of mohair or other animal fibre intertwined. By varying the denier of the strands or by using more than two strands, the proportion of one type to the other 15 may be varied, but there should be at least twenty-five percent of each, and I prefer the mohair to make up from 50 to 75% of the thread. The acetate strand may be of the fuzzy type already described and may be pigmented if desired. These strands are, as is usual, separately 20 twisted and then twisted together so as to give a balanced twist.

The filling thread may be spun from fibres of 25 mohair and cellulose acetate in suitable proportion, the amounts of which are of the same order, and here also the acetate may be pigmented black or white or in colors.

The resulting fabric, besides having a pleasing 30 distinctive appearance and feel, is non-irritant, holds its shape well when pressed with heat and moisture as in tailoring but does not retain incidental creasing due to folding or mussing. This is due to the inherent resiliency of the mohair. At the same time, it has a striking advantage in 35 the uniform slight amount of shrinkage which it has in both directions.

The amount of cellulose acetate in the combined thread is sufficient to keep the yarn when 40 wet from shrinking to an undue extent.

What I claim is:

1. A fabric comprising warp and woof threads, one being of cellulose acetate, and the other being twisted from at least two strands, one being of mohair and the other of cellulose acetate, the 45 cellulose acetate strands comprising multiple filaments the outer ones of which are broken, whereby the strand has a fuzzy surface.

2. A fabric consisting of warp and woof threads, the threads extending in one direction 50 being composed predominantly of cellulose acetate and the threads extending in the other direction being composed of intertwined cellulose acetate filaments and natural animal fibres selected from the group consisting of hair and wool. 55

3. A fabric consisting of warp and woof threads, the threads extending in one direction being composed predominantly of cellulose acetate and the threads extending in the other direction being composed of intertwined cellulose acetate filaments and natural animal fibres selected from the group consisting of hair and wool, the cellulose acetate filaments and the animal fibres each constituting at least 25% of the threads extending in the second direction.
4. A fabric consisting of warp and woof threads, the threads extending in one direction being composed predominantly of cellulose acetate and the threads extending in the other direction being composed of intertwined cellulose acetate filaments and wool fibres.
5. A fabric consisting of warp and woof threads, the threads extending in one direction being composed predominantly of cellulose acetate and the threads extending in the other direction being composed of intertwined cellulose acetate filaments and mohair fibres.
6. A fabric consisting of warp and woof

threads, the threads extending in one direction being predominantly of cellulose acetate and the threads extending in the other direction being twisted from at least two strands, one strand being of cellulose acetate filaments and the other strand being of animal fibres selected from the group consisting of hair and wool.

7. A fabric consisting of warp and woof threads, the threads extending in one direction being predominantly of cellulose acetate and the threads extending in the other direction being twisted from at least two strands, one strand being of cellulose acetate filaments and the other strand of wool fibres.

8. A fabric consisting of warp and woof threads, the threads extending in one direction being predominantly of cellulose acetate and the threads extending in the other direction being twisted from at least two strands, one strand being of cellulose acetate filaments and the other strand of mohair fibres.

ASHTON M. TENNEY.